

April 8, 1952

A. JOHNSON ET AL

2,592,154

CELLULOOSIC TEXTILE FABRIC

Filed Jan. 8, 1948

FORM A COMPOSITE YARN BY WINDING ALKALI  
SOLUBLE ALGINATE YARN WITH COTTON STAPLE YARN. *Fig. 4.*

↓  
WEAVE THE COMPOSITE YARN INTO A FABRIC.

↓  
WASH THE FABRIC IN AN ALKALINE BATH TO DISSOLVE  
THE ALGINATE YARN.

*Fig. 1.*



*Fig. 2.*



*Fig. 3.*

INVENTORS.  
ARTHUR JOHNSON &  
JOHN BAMBER SPEAKMAN

*Stebbins, Blenko & Welt.*  
*Attyp.*

## UNITED STATES PATENT OFFICE

2,592,154

## CELLULOSIC TEXTILE FABRIC

Arthur Johnson and John Bamber Speakman,  
Leeds, England, assignors to Alginic Industries  
Limited, Maidenhead, England, a British com-  
pany

Application January 8, 1948, Serial No. 1,150  
In Great Britain April 11, 1941

2 Claims. (Cl. 28—72)

1

This application is a continuation-in-part of our copending application Serial No. 571,758, filed January 8, 1945, now Patent No. 2,435,543, which in turn is a division of our application Serial No. 450,012, filed July 7, 1942, now abandoned.

This invention comprises improvements in or relating to cellulosic textile fabrics.

In the weaving of textile fabrics it is known to use yarns twisted with cotton threads, which latter are intended to remain in the fabric only temporarily, and after weaving to remove the cotton by treatment with sulphuric acid, drying and baking, whereby the cotton is carbonised and reduced to a powder, which is easily dusted out. Cotton and wool yarns are twisted together in such a sense as to leave the wool yarn in the two-fold thread either twistless or deficient in twist so that when the cotton is removed in carbonising a soft and lustrous fabric is obtained. The process is applicable only to wool fibres but even they are liable to be damaged to some extent by the use of acid, so that the avoidance of the use of acid is a matter of importance.

The present invention relates to the production of fabrics from yarns of cellulosic staple fibres of such fineness as is not normally capable of being made into fabric. In particular the invention comprises a woven cellulose staple fibre fabric comprising yarn of such fineness that it is incapable by itself of withstanding the strains imposed in weaving. The invention is not, however, limited to woven fabrics but includes knitted and lace fabrics.

It is found that soluble alginic fibres can be employed successfully with all cellulosic fibres and not simply with the acid-resisting wool fibres which are sometimes used twisted up with cotton in processes which involve subsequent removal of the cotton by acid. Soluble alginic fibres are known in themselves; for example fibres of alginic acid and metal alginates like calcium alginate are known, both types being soluble in soap, soda and other alkaline solutions.

The invention further comprises a process for the manufacture of a woven or knitted or lace fabric characterised by producing composite yarn by twisting together soluble alginic fibres and cellulosic staple textile fibres of such fineness as is too weak to be handled by itself in making the fabric, employing such composite yarn, with or without other yarn, in making the fabric and thereafter dissolving the said soluble alginic fibres out of the fabric so as to set the fine cellulosic staple fibres free.

2

Many alginic fibres, such for example as fibres of calcium alginate, are soluble in an aqueous solution of soap or sodium carbonate or can be converted to alginic acid by treating with an acid of such strength as will not injure wool fibres, in which converted state they are soluble in, say, sodium carbonate, and it is this readily soluble property of many alginic fibres which is utilised according to the present invention and the expression "soluble alginic fibres" is to be understood accordingly.

The phrase "fibres" is used in this specification as including both long filaments and relatively short fibres, and where short fibres are referred to specifically they are referred to as staple fibres.

The lower limits of fineness with which yarns of staple cellulosic fibres can be spun, or woven, depend upon the nature of the fibres, and are herein specified in terms of yards per pound of yarn, in order to avoid any confusion between the differing manners of reckoning the fineness of cotton or linen or viscose staple fibres, which are the three commercially important kinds of such fibres. The finest linen yarns producible on a commercial scale have a length of about 90,000 yards per pound weight. Such yarns are too weak to be woven in a power loom, the finest linen yarns for weaving having a length of about 48,000 yards per pound.

The finest cotton yarns which can be spun have a length of as much as 336,000 yards per pound, but cotton of such fineness cannot normally be woven in a power loom, the finest cotton for this purpose being about 134,000 yards per pound.

The finest viscose staple fibre yarns which can be spun are 56,000 yards per pound but such yarns cannot be woven normally in a power loom, the finest yarn for the purpose being about 22,400 yards per pound.

According to one feature of this invention, linen yarn finer than 48,000 yards per pound or cotton yarn finer than 134,000 yards per pound or viscose staple fibre yarn finer than 22,400 yards per pound is twisted with soluble alginate yarn to produce a composite yarn capable of being woven on a power loom notwithstanding the fact that the yarn by itself could not be so woven and after weaving the alginate yarn is removed by a weak alkaline scour to leave a fabric finer than could otherwise be produced.

The cellulosic fibres in the composite yarn may, moreover, be substantially untwisted, or less twisted than would be necessary to withstand weaving stresses whereby a softer or more lus-

## 3

trous or stronger fabric is produced. In explanation of this it may be pointed out that certain fabrics are distinguished by their soft and full-handling properties. Although these tactile qualities may often be enhanced by suitable finishing processes, they are largely determined by the structure of the yarns from which the fabrics are made. Ordinary yarns must, of necessity, be twisted sufficiently to withstand the strains imposed in weaving, but softness decreases as the twist increases. Thus certain yarns when twisted sufficiently to be suitable for weaving may contain so much twist as to prevent the desired degree of softness being realised in the finished fabric. In the case where, according to the present invention a yarn of cellulosic fibres is twisted to form a composite thread with soluble alginic yarn the alkaline wash removes the alginic fibres and if the composite yarn has been twisted in such a manner that, in twisting, the original twist in the cellulosic fibres is practically or wholly untwisted, the cellulosic fibres which remain after washing will be twistless, or at all events less twisted than would be necessary for weaving or otherwise making into fabric by themselves and the resulting fabric will be softer. Moreover, such a process gives a fabric possessing a higher lustre than one composed of yarns twisted so as to withstand weaving, and the same principle can, of course, be applied to increase the lustre of individual threads in a fabric, such as coloured and uncoloured striping threads. It will be observed that the word "yarn" is employed in a broad sense as including groups of fibres or filaments which are twistless, such as those left twistless in the finished fabric, according to this invention.

The effects according to the present invention can be obtained with ordinary textile fibres of all kinds, including cotton, linen and viscose staple, and not simply acid-resistant fibres such as wool and mohair. An important series of new types of fabric is thus made available for the first time.

One important advantage of the manufacture of fabrics in accordance with this invention from threads which are twistless or little twisted after removal of the soluble alginic yarn is that a twistless or little twisted thread may be made to develop the maximum strength of the fibres in the woven fabric. Thus, for example, a fabric in which both warp and weft are woven from cotton in such a way as to leave the fibres twistless or little twisted in the finished fabric may for a given weight be as strong as or even stronger than a fabric made from cotton yarns having normal twist. The cotton threads could not be woven by themselves without being twisted, but by the use of the alginic yarn for binding them together during weaving, the weaving operation becomes possible with the twistless or little-twisted cotton.

The preferred form in which the soluble alginic threads are employed in accordance with this invention is in the form of calcium alginate which is soluble in soap or soda solutions. When calcium alginate is used the attack by the soap leads to the production of an insoluble metal soap, for example calcium oleate. In cases where the presence of this insoluble metal soap would be objectionable, say in dyeing, other alkaline scours can be substituted, for example, fatty alcohol sulphates with soda or a mixture of soap, soda and one of the known polymers of alkali phosphates which prevent precipitation of calcium soaps.

## 4

Again the alginic yarn may be converted to alginic acid by a mild acid treatment followed by removal in sodium carbonate solution and this will ensure that no calcium soaps remain in the fabric after treatment.

In the accompanying drawings which illustrate our invention diagrammatically.

Figure 1 is a diagram of one form of fibre with a twisted cellulose component.

Figure 2 is a diagram of a second form with the cellulose component untwisted,

Figure 3 represents a fabric made by weaving the yarn shown in Figure 1 into a fabric, and

Figure 4 is a flow sheet illustrating the steps of our process.

To produce the yarn shown in Figure 1 the cellulose component, which may be of linen, cotton or viscose staple fibre, and is indicated by the fibres 11, is first spun into yarn by itself.

Thereafter it is twisted together with yarn of calcium alginate, shown by the continuous filament 12. It will be noted that this has been done so that the cellulosic component remains twisted in the combined yarn and so if the yarn is woven or knitted or otherwise made into fabric, on removal of the calcium alginate in an alkaline bath the cellulosic constituent will retain its twisted formation.

In Figure 2 the cellulosic constituent 13 is untwisted or substantially so and the continuous alginic constituent 14 is wound round it and keeps it together. This is effected by winding together the alginate fibre yarn and the cellulosic yarn with a direction of twist opposite to that

initially given to the cellulosic yarn when it is first spun, so that in twisting them together the initial twist is taken out of the cellulosic yarn.

The following examples are illustrative of manufacture in accordance with the invention:

*Example I*

A fine linen yarn is spun of such fineness as to have a length of 90,000 yards per pound weight. This is twisted with a calcium alginate filament

of 100 denier which gives the combined yarn sufficient strength to be woven on a power loom. The direction of twisting is such as to retain the twist of the linen yarn as shown in Figure 1. A fabric is woven therefrom and after weaving the

calcium alginate fibres are dissolved out by means of an alkaline scour comprising a weak sodium carbonate solution containing also a small percentage of soap and of "Calgon" (sodium hexametaphosphate). The result is a linen fabric which is lighter than can be produced by usual commercial methods in power looms.

*Example II*

A fine cotton yarn is spun having a fineness of 200,000 yards per pound and is twisted with calcium alginate yarn of a fineness of 100 denier, the twist of the cotton being retained as in Figure 1. This is woven and after dissolving out the alginic constituent as described in Example

I the result is a cotton fabric of peculiar fineness. Very fine cotton fabrics can be woven without such composite yarns but it is not normally possible, by ordinary commercial methods, to produce a woven fabric of such fineness as is here indicated.

*Example III*

Viscose staple fibre is taken and spun into a fine yarn having a length of 56,000 yards per pound. This represents a finer yarn than can

normally be woven; it is twisted with an alginate filament having a fineness of 100 denier so as to retain the twist of the viscose staple fibre, and woven, after which the alginate yarn is removed as described in Example I and a stable-fibre viscose fabric results of great lightness, such as could not heretofore be produced.

*Example IV*

A composite yarn is produced consisting of one thread of  $1/30$ 's cotton, which may be mercerised, twisted with a 100 denier calcium alginate rayon, so that the cotton thread is in a twistless form. This composite thread is used as a striping thread in a fabric, the alginate rayon enabling the twistless cotton to withstand the weaving strains. After weaving, the supporting thread of calcium alginate is removed by means of the normal alkaline scour which is used in finishing fabrics and leaves the  $1/30$ 's twistless cotton stripe. This cotton stripe will be found to have far greater covering power and to be much more prominent and lustrous than a stripe woven from an ordinary twisted mercerised cotton. Such a twisted cotton consists normally of two threads of  $1/60$ 's cotton twisted together with twenty-three turns per inch and the twist in the cotton detracts from its covering power and from its lustre as compared with the twistless  $1/30$ 's in accordance with the present invention.

*Example V*

A fabric is woven in which the warp and the weft both consist of  $1/30$ 's cotton yarn twisted with a 100 denier calcium alginate rayon to form a composite thread in which the cotton portion is twistless. After weaving, the calcium alginate threads are removed by the alkaline scour leaving a fabric entirely consisting of  $1/30$ 's twistless cotton threads. Such threads press flat and, providing the residual threads are packed as tightly as possible, they afford the maximum possible strength to the fabric and owing to their flattened form they leave smaller apertures between the threads in the finished fabric. Such a fabric is stronger, thinner and requires less "dope" to fill the apertures than an equivalent fabric woven from ordinary twisted cotton.

*Example VI*

A composite yarn similar to that of Example IV of cotton and alginate fibres, the cotton fibres being untwisted as shown in Figure 2 hereof, is taken, and woven into a compound fabric with other yarns so that the composite yarn forms the centre portion of the fabric and is inter-

woven with outer cloth portions of plain cotton fabric so that the untwisted yarn constitutes a soft filling between the outer cloths when the soluble alginic fibres have been dissolved.

5

*Example VII*

Composite cotton and alginate yarn such as is referred to in Examples IV to VI is taken and woven as wadding threads on the surface of a cotton fabric. After removal of the alginic yarn by scouring, as already described, the result is a very soft layer on the face of the fabric. This may be produced either on one face or both faces of the fabric.

15

We claim:

1. A woven fabric substantially consisting of singles cotton yarn having a fineness greater than 134,000 yards per pound, wound with alginate yarn of between 50 and 100 denier, the alginate 20 yarn being soluble in an alkaline bath without injury to the cotton yarn.
2. A process of making woven fabrics which comprises winding alkali soluble alginate yarn having a fineness of between 50 and 100 denier 25 with cotton staple yarn having a fineness greater than 134,000 yards per pound to form a composite yarn, weaving a fabric from the composite yarn and thereafter washing the fabric in an alkaline bath to dissolve the alginate yarn.

30

ARTHUR JOHNSON.

JOHN BAMBER SPEAKMAN.

REFERENCES CITED

The following references are of record in the 35 file of this patent:

UNITED STATES PATENTS

| Number       | Name      | Date          |
|--------------|-----------|---------------|
| 362,318      | Scheppers | May 3, 1887   |
| 40 1,021,712 | Wilkinson | Mar. 26, 1912 |
| 2,011,916    | Simonds   | Aug. 20, 1935 |
| 2,159,265    | Gash      | May 23, 1939  |
| 2,332,738    | Meade     | Oct. 26, 1943 |
| 2,435,543    | Johnson   | Feb. 3, 1948  |

45

OTHER REFERENCES

"American Cotton Handbook," first edition, Barnes Printing Co., New York, 1941, page 512. (Copy in Div. 21.)

50 "International Library of Technology, Yarns, Cloth Rooms, Mill Eng'ng, Reeling, Baling, Winding," International Textbook Co., Scranton, Pa. 1906 (pages 16 and 17). (Copy in Div. 21.)

Bendure et al., "American's Fabrics," Macmillan Co., 1947, New York, page 303. (Copy in Div. 21.)